

## UNITED STATES PATENT OFFICE

2,421,693

## IMIDAZOLONE COLOR FORMERS

Benjamin Ramage Harriman, Binghamton, N. Y.,  
assignor to General Aniline & Film Corporation,  
New York, N. Y., a corporation of Delaware

No Drawing. Application September 16, 1944,  
Serial No. 554,541

11 Claims. (Cl. 95—6)

1

The present invention relates to color photography and, more particularly, to color forming or coupling components suitable for use in the process of color forming development, in which color is produced in a photographic emulsion layer by the action of an oxidation product of the photographic developer on a dyestuff component present in said layer during development.

The present invention is an improvement on the process of color forming development first described in United States Patents No. 1,055,155 and No. 1,102,028 to Fischer, in accordance with which a color forming development component which is incorporated either in the photographic emulsion layer or in the development bath, and which when the emulsion layer is developed by means of a developer containing free amino groups, for instance, aromatic diamines, especially the mono- or unsymmetrically di-substituted ones, like p-dimethylaminoaniline, or methoxy-p-dimethylaminoaniline, couples with the oxidation product of the photographic developer to form a dyestuff at the points where a silver image is produced. In accordance with more recent developments of this process, it is preferable to employ, as the color forming or coupling component, a compound which is non-diffusing in the photographic emulsion, rather than one which is soluble in the photographic developing solution. This is particularly true if several differently sensitized emulsion layers are cast on a single support, as is the case in the so-called integral tripack photographic color films, since in such case, any wandering or diffusing of a color coupling component from the emulsion layer in which it is incorporated to another will cause inaccurate color rendition.

In such color forming development process, it has been customary to employ various pyrazolones for the production of red or magenta pictures. The coupling takes place at points where a silver image is formed between the oxidation product of the color forming developer and the active methylene group of the pyrazolone ring. It is recognized, however, that many of the pyrazolones that may be employed as magenta color coupling components have a relatively high blue adsorption and therefore are not entirely satisfactory as color forming components.

2

It is an object of the present invention to provide a new type of color forming components, closely related to the pyrazolones, in which the heterocyclic ring is slightly modified without destroying the active methylene group. Other and further objects will become apparent as the following description progresses.

I have discovered that the imidazolones are valuable color forming components and that many imidazolones may be obtained which produce particularly valuable magenta colors on coupling with the oxidation product of a color forming developer and that such coupling, between the active methylene group of the imidazolone ring and the oxidation product of the color former developer, is readily brought about by the usual color forming development processes.

The imidazolones which I have found are particularly valuable as color forming components and may be represented by the following general formula:



in which R stands for hydrogen, alkyl, aryl, aralkyl, or acyl, which may be further substituted; for instance, by amino, acyl, acylamino, sulfo, nitro, hydroxy, amino sulfo, etc.; R' stands for the residue of a pyridine, quinoline or isoquinoline radical, which may be further substituted; and X is a negative substituent, such as halogen, carboxylic or sulfonic acid group, or the like.

The imidazolones which I employ as color forming components may readily be prepared by known methods of synthesis. A convenient method by which to prepare these imidazolones is to employ 2-amino-pyridine or quinoline as the starting material and react this with an  $\alpha$ -halogenated acyl halide, for instance, monochloroacetic acid chloride. This reaction may readily be carried out in dry ether or other anhydrous solvent at room temperatures. A hydrochloride is formed first and this is dumped in water so that hydrochloric acid is split off and the chloro acyl amino compound precipitates. This material

3

may then be separated by filtration, dried, dissolved in a suitable solvent, for instance, nitrobenzene, and heated slightly above its melting point, preferably 120-180° C. On such heating, the nitrogen atom of the pyridine or quinoline ring is quaternized and the amino group cyclized with the resulting formation of an imidazolone ring. The above series of reactions takes place in accordance with the following Equation I:

Eq. I



and is particularly valuable in case 2-amino-quinoline is employed as a starting material.

An alternative method of preparing imidazolones, suitable for use in accordance with the present invention, and which is slightly more satisfactory in case 2-amino-pyridine is employed as a starting material, but which does not function so well in case quinolines are employed, is to react the 2-amino-pyridine with the sodium salt of monochloroacetic acid, thus quaternizing the amino group of the pyridine ring and forming a cyclic salt. The thus-obtained cyclic salt may be dehydrated readily in accordance with conventional procedures to form thereby an imidazolone ring. This method of synthesis may be represented by the following Equation II:

Eq. II



Other methods of synthesis will also suggest themselves to those skilled in the art. Thus, if desired, the imidazolones may be obtained directly by heating together substantially equal molecular amounts of 2-amino-pyridine and an ester

4

of monochloroacetic acid, as represented by the following Equation III:

Eq. III



The solubility of the imidazolones prepared as described above may be modified by the nature of the substituents thereon. Thus, a convenient method of obtaining non-diffusibility in the imidazolone is to introduce a long chain alkyl substituent on the nitrogen atom in 1-position. An imidazolone containing such a substituent is readily obtained by employing, as a starting material, a pyridine or a 2-amino-pyridine or quinoline in which the amino group contains a long chain alkyl group. Non-diffusibility is obtained when the alkyl group of the amine contains 8 or more carbon atoms.

In a similar manner, the particular shade or color obtained may be influenced, to a large extent, by the nature of the substituents in the pyridine ring.

The following specific examples are illustrative of the present invention:

#### Example 1

2-keto-4-chloro-imidazo[1,2-a] pyridine, prepared as outlined above in Equation II, was incorporated in a photographic emulsion in the usual manner by dissolving the same in an aqueous solution, for instance, by dissolving a small amount, say 8 grams, in 100 ml. of water. The thus obtained photographic emulsion was cast on a suitable support to produce a photographic film, which after exposure and development with a color forming developer, p-diethylaminoaniline, gave a magenta picture. The color coupling component, however, was diffusible from the photographic emulsion.

In order to overcome this diffusibility in the photographic emulsion, a similar compound, 1-octadecyl-2-keto-4-chloro-imidazo[1,2-a] pyridine, was prepared in the manner outlined under Equation II above, substituting 2-octadecylpyridine for the 2-aminopyridine there mentioned. 4.0 grams of this product were dissolved in 100 ml. of H<sub>2</sub>O and incorporated in a photographic emulsion. The thus obtained color former was non-diffusing in the emulsion and the emulsion could be cast on a suitable support, in accordance with conventional practice, to produce a photographic film. After exposure and development of the film with a color forming developer, p-diethylaminoaniline, a magenta picture was obtained.

#### Example 2

2-keto-4-chloro-imidazo[1,2-a] quinoline was prepared as outlined in Equation I above. This material was incorporated in a photographic emulsion in a conventional way, for instance, as outlined under Example 1 above, and the emulsion cast on a suitable support, in accordance with conventional practice, to produce a photographic film. After exposure and development with a color forming developer, p-diethylaminoaniline, a magenta picture was obtained.

The color former was subject to the objection that it was diffusible from the photographic emulsion. In order to overcome this difficulty, a similar color former, 1-octadecyl-2-keto-4-chloro-imidazo [1,2-a] quinoline, was prepared in accordance with the method outlined in Equation I above, substituting 2-octadecylaminoquinoline for the 2-aminoquinoline there specified. This color former was sulfonated in order to improve its solubility and was then dissolved in an aqueous solution and added to a photographic emulsion in the manner specified in Example I above. The color former was found to be non-diffusing in the photographic emulsion. The emulsion containing the color former was cast on a suitable support, in accordance with conventional practice, to produce a photographic film. After development with a color forming developer, p-diethylaminoaniline, a magenta picture was obtained.

Still another method of overcoming the difficulty of diffusion is to treat the 2-keto-4-chloro-imidazo [1,2-a] quinoline with a long chain acyl chloride, for instance, with stearyl chloride which results in the introduction of a stearyl group on the nitrogen in the 1-position to give 1-stearyl-2-keto-4-chloro-imidazo [1,2-a] quinoline.

The introduction of a long chain acyl group into the 1-position of the imidazo [1,2-a] pyridine compound does not always proceed satisfactorily by the method just described, i. e., treating the imidazo [1,2-a] pyridine compound with an acyl halide.

An alternative method that in most cases gives better yields and more easily purifiable products consists in treating an inner cyclic salt, referred to above, (B) in Equation II, with a long chain aliphatic acid anhydride, for example stearic acid anhydride. Thus, gently warming together



and stearic acid anhydride resulted in an almost quantitative yield of



which was a blue magenta, non-diffusing color former. When this was incorporated in an emulsion, and the resulting photographic element exposed and developed with the coupling developer p-amino-diethylaniline, a blue magenta image was obtained, which had a spectral absorption maximum at 560 mu.

Dyes with absorption maxima close to 560 mu. were obtained from 2-keto-4-chloro-imidazo [1,2-a] pyridines substituted in the 1-position by hydrogen, alkyl, or acyl, and in the pyridine ring by hydrogen, methyl, nitro, chloro, amino, etc.

Dyes with absorption maxima close to 580 mu. were obtained from 2-keto-4-chloro-imidazo [1,2-a] quinolines substituted in the 1-position by hydrogen, alkyl, or acyl, and in the quinoline ring by hydrogen, methyl, nitro, chloro, amino, etc.

Other specific color formers of the type embodied in the present invention are listed below in tabular form, together with the spectral absorption maximum for the dyes produced on color forming development with p-aminodiethylaniline of exposed photographic gelatine silver halide emulsions in which these color formers had been incorporated as outlined above.

## Example 3

| Color Former                                                 | Spectral Absorption Maximum |
|--------------------------------------------------------------|-----------------------------|
| 1-acetyl-2-keto-4-acetate-9-methyl-imidazo [1,2-a] quinoline | 580 Mu.                     |

## Example 4

| Color Former                                        | Spectral Absorption Maximum |
|-----------------------------------------------------|-----------------------------|
| 1-acetyl-2-keto-4-acetate imidazo [1,2-a] quinoline | 580 Mu.                     |

## Example 5

| Color Former                                      | Spectral Absorption Maximum |
|---------------------------------------------------|-----------------------------|
| 2-keto-4-chloro-5-methyl-imidazo-[1,2-a] pyridine | 560 Mu.                     |

## Example 6

| Color Former                                                      | Spectral Absorption Maximum |
|-------------------------------------------------------------------|-----------------------------|
| 1-propionyl-2-keto-4-propionate-6-chloro-imidazo [1,2-a] pyridine | 560 Mu.                     |

## 7 Example 7

| Color Former                                                   | Spectral Absorption Maximum |
|----------------------------------------------------------------|-----------------------------|
| 1-acetyl-2-keto-4-acetate-6-nitro-imidazo-[1,2-a] pyridine<br> |                             |

## 8 Example 8

| Color Former                                     | Spectral Absorption Maximum |
|--------------------------------------------------|-----------------------------|
| 2-keto-4-chloro-imidazo [1,2-a] isoquinoline<br> | 580 Mu.                     |

## 9 Example 9

| Color Former                                         | Spectral Absorption Maximum |
|------------------------------------------------------|-----------------------------|
| 2-keto-4-chloro-6-amino-imidazo [1,2-a] pyridine<br> |                             |

I claim:

1. A photographic element comprising a silver halide photographic emulsion containing as a color forming development component an imidazolone of the formula



wherein R' represents the residue of a member of the group consisting of pyridine, quinoline and isoquinoline radicals, R represents a member of the group consisting of H, alkyl, aryl, aralkyl and acyl, and X is a negative ion of a quaternary ammonium salt.

2. A photographic element comprising a silver halide photographic emulsion containing as a color forming development component an imidazolone of the formula



wherein the pyridine ring may bear substituents selected from the group consisting of lower alkyl, nitro, halo and amino groups, and wherein X is a negative ion of a quaternary ammonium salt.

3. The method of producing color pictures which comprises developing a silver halide photographic emulsion with a color forming developer in the presence of a color forming development component of the formula

10



15 wherein R' represents the residue of a member of the group consisting of pyridine, quinoline and isoquinoline radicals, R represents a member of the group consisting of H, alkyl, aryl, aralkyl, and acyl, and X is a negative ion of a quaternary ammonium salt.

20 4. The method of producing color pictures which comprises developing a silver halide photographic emulsion with a color forming developer in the presence of a color forming development component of the formula

30



wherein the pyridine ring may bear substituents selected from the group consisting of lower alkyl, nitro, halo and amino groups, and wherein X is a negative ion of a quaternary ammonium salt, and R is a member of the group consisting of H, alkyl, aryl, aralkyl, and acyl.

45 5. A photographic element comprising a silver halide photographic emulsion containing as a color forming development component an imidazolone of the formula

50



55 wherein the quinoline radical may bear substituents selected from the group consisting of lower alkyl, nitro, halo and amino groups and wherein X is a negative ion of a quaternary ammonium salt, and R is a member of the group consisting of H, alkyl, aryl, aralkyl, and acyl.

60 6. The method of producing color pictures which comprises developing a silver halide photographic emulsion with a color forming developer in the presence of a color forming development component of the formula

65



70 wherein the quinoline radical may bear substituents selected from the group consisting of lower alkyl, nitro, halo and amino groups, and wherein X is a negative ion of a quaternary ammonium salt, and R is a member of the group consisting of H, alkyl, aryl, aralkyl, and acyl.

75 7. A photographic element comprising a silver halide photographic emulsion containing as a

9

color forming development component an imidazolone of the formula



wherein the quinoline residue may bear substituents selected from the group consisting of lower alkyl, nitro, halo and amino groups, and wherein X is a negative ion of a quaternary ammonium salt, and R is a member of the group consisting of H, alkyl, aryl, aralkyl, and acyl.

8. The method of producing color pictures which comprises developing a silver halide photographic emulsion with a color forming developer in the presence of a color forming development component of the formula



wherein the quinoline residue may bear substituents selected from the group consisting of lower alkyl, nitro, halo and amino groups, and wherein X is a negative ion of a quaternary ammonium salt, and R is a member of the group consisting of H, alkyl, aryl, aralkyl, and acyl.

9. A photographic element comprising a silver halide photographic emulsion containing as a color forming development component an imidazolone of the formula



wherein R' represents the residue of a member of the group consisting of pyridine, quinoline and isoquinoline radicals, R is a long chain alkyl group, and X is a negative ion of a quaternary ammonium salt.

10

10. The method of producing color pictures which comprises developing a silver halide photographic emulsion with a color forming developer in the presence of a color forming development component of the formula



wherein R' represents the residue of a member of the group consisting of pyridine, quinoline and isoquinoline radicals, R is a long chain alkyl group, and X is a negative ion of a quaternary ammonium salt.

11. The method of producing color pictures which comprises developing a photographic silver halide emulsion with a primary aromatic amino developer in the presence of a color coupler having the formula



wherein X is a negative ion.

BENJAMIN RAMAGE HARRIMAN.

#### REFERENCES CITED

The following references are of record in the file of this patent:

#### UNITED STATES PATENTS

| Number       | Name                   | Date          |
|--------------|------------------------|---------------|
| 40 2,154,918 | Schneider et al. ----- | Apr. 18, 1939 |
| 2,186,736    | Schneider et al. ----- | Jan. 9, 1940  |
| 2,293,004    | Lohus -----            | Aug. 11, 1942 |
| 2,343,704    | Porter et al. -----    | Mar. 7, 1944  |
| 2,350,812    | Peterson -----         | June 6, 1944  |

#### FOREIGN PATENTS

| Number  | Country             | Date          |
|---------|---------------------|---------------|
| 478,986 | Great Britain ----- | Jan. 24, 1938 |
| 511,790 | Great Britain ----- | Aug. 24, 1939 |
| 519,695 | Great Britain ----- | Apr. 3, 1940  |